

Oct. 16, 1923.

1,471,052

W. D. MOORE

# METHOD OF AND APPARATUS FOR CENTRIFUGALLY CASTING METAL BODIES

Filed March 1, 1923



Oct. 16, 1923.

1,471,052

W. D. MOORE

METHOD OF AND APPARATUS FOR CENTRIFUGALLY CASTING METAL BODIES

Filed March 1, 1923

4 Sheets-Sheet 2



Oct. 16, 1923.

1,471,052

W. D. MOORE

METHOD OF AND APPARATUS FOR CENTRIFUGALLY CASTING METAL BODIES

Filed March 1, 1923

4 Sheets-Sheet 3



INVENTOR

William D. Moore

BY

Moers, Cavanaugh, Whitehead  
ATTORNEYS

Oct. 16, 1923.

1,471,052

W. D. MOORE

METHOD OF AND APPARATUS FOR CENTRIFUGALLY CASTING METAL BODIES

Filed March 1, 1923

4 Sheets-Sheet 4



INVENTOR  
William D. Moore

BY  
Meyers, Cavanagh & Whitehead  
ATTORNEYS

## UNITED STATES PATENT OFFICE.

WILLIAM D. MOORE, OF BIRMINGHAM, ALABAMA, ASSIGNOR TO AMERICAN CAST IRON PIPE COMPANY, OF BIRMINGHAM, ALABAMA, A CORPORATION OF GEORGIA.

## METHOD OF AND APPARATUS FOR CENTRIFUGALLY CASTING METAL BODIES.

Application filed March 1, 1923. Serial No. 622,082.

To all whom it may concern:

Be it known that I, WILLIAM D. MOORE, a citizen of the United States, and resident of Birmingham, in the county of Jefferson and State of Alabama, have invented certain new and useful Improvements in Methods of and Apparatus for Centrifugally Casting Metal Bodies, of which the following is a specification.

10 This invention relates to the art of making metal castings, and more particularly to a method and apparatus for centrifugally casting hollow metal bodies, and has special reference to the making of cylindrical castings such as ferrous pipe in a centrifugally operated mold.

15 The prime desideratum of the present invention comprehends the provision of a method of and apparatus for centrifugally casting hollow metal bodies in preferably refractory molds, and more particularly in unbaked or "green" sand molds, for the making especially of commercial ferrous metal pipe with or without bell and spigot 20 ends in an economical and efficient manner.

25 As is well known, a number of methods for centrifugally casting hollow metal bodies such as pipe have hitherto been proposed consisting variously in rotating about a horizontal, vertical or an inclined axis or a combination of these, either a metal hot or cooled mold or a refractory such as a sand or clay mold, into which mold the molten metal is discharged for distribution 30 by centrifugal action about the inner wall thereof to form the hollow casting or pipe. The prior practice of these methods has been attended with numerous disadvantages, either from the aspect of the difficulties involved in carrying out the steps of the 35 method, or from that of the objectionable cost of installation and renewal of the apparatus employed, or the added expense and inconvenience of special treatment of the 40 castings required, or the structural defects of the castings produced, or the relatively large cost of the metal mixtures or alloys necessitated by the limitations or requirements of the process; and due to these difficulties encountered, centrifugal casting proc-

esses have not been generally adopted by the trade.

45 In the casting centrifugally of pipe structures with the use of the metal or so-called permanent mold, the molten metal is supplied to the mold with the latter either heated or cold, depending upon the process adopted. Where heated molds have been employed, it has been found that, aside from the objections attending the heating of the 50 mold and the handling of the same, the extraction of the casting from the mold is very difficult of accomplishment, and the casting produced is too brittle for commercial service. Where a cold or chilled metal mold is 55 employed, the casting produced must undergo expensive annealing treatment at high temperatures, and the casting product obtained after chilling and annealing, although apparently structurally adequate, is 60 defectively weak, especially in its resistance to corrosion. It is well known, for example, that annealing at high temperatures causes changes in the characteristics of the 65 metal; and that the crystalline structure of the metal consisting of a matrix of pearlite largely interspersed with flakes of graphite, upon which crystalline structure the resistance to corrosion is largely dependent, 70 breaks down as a result of the annealing treatment into grains of iron with flakes of amorphous carbon scattered through the structure. The use of the cold mold further necessitates a high silicon content of 75 the metal, and hence an expensive metal mixture. The metal molds, moreover, either of the hot or cold type, are comparatively 80 expensive and relatively short-lived, and the cost of renewing or replacing the mold adds a fairly large increment to the cost of production of the pipe. Thus the metal mold centrifugal casting process is found to be 85 comparatively uneconomical, and the product is found unable to withstand that degree of corrosion and deterioration dictated 90 by its intended industrial use.

95 In the centrifugal casting of hollow bodies with the use of sand molds, the molten metal is discharged into a flask lined with sand provided with a facing on the in- 100

ner surface thereof, one process comprehending the utilization of a "green" or unbaked sand lining, and another process including the use of a baked or dry sand lining. Of these the "green" sand mold process has been found to be the more economical due for example to the elimination of the time consumed and in the cost of baking the mold in the dry sand mold method, and permits of obtaining a better casting product resulting from a number of factors. The castings obtained from the centrifugally operated "green" sand mold combine the desirable properties of ordinary sand cast metal such as the superior resistance of the casting to corrosion and other actions which tend to disintegrate the metal and shorten the life of the pipe, with the high qualities of centrifugally cast products, such as the greater density and solidity and consequent greater strength. Although the "green" sand mold process is thus capable of yielding a superior metal pipe or tubular product, the processes heretofore proposed have not met with commercial adoption due to the difficulties that have been met with in centrifugally casting on sand molds, which difficulties heretofore have been regarded as unavoidable and have not been successfully solved.

Among the more prominent problems presented in the art of centrifugally casting on refractory molds were, for example, the difficulties of causing the metal to flow evenly on a sand mold and securing an even distribution of the molten metal in the mold to obtain a uniform and homogeneous product; the further difficulty of preventing the cutting and washing of the sand by the action of the molten metal discharging into and flowing through the mold; the further difficulty presented especially in "green" sand molds of producing a clean casting without pocketed or honeycomb defects; the further problems governing the use of facings which were not properly united or associated with the sand lining, and which were picked up by and washed and carried along with the flowing metal, resulting not only in leaving blemishes on the surface of the casting, but in the production of a prohibitive amount of scruff; and such further mechanical objections as the instability of the sand lining when the mold is subjected to rotation at high speeds. To obviate these and other defects and drawbacks, as will appear further hereinafter, and to successfully produce economically the desired casting product obtained in a centrifugal sand mold, is a prime desideratum of my present invention.

The principal objects of my present invention may be said to include the provision of a method of and apparatus for centrifugally casting hollow metal bodies in refractory molds, in which the molten metal is

so introduced in a rotary mold and the mold so coordinately operated as to effect a uniform distribution of the metal in the mold to produce a uniform and homogeneous casting; the further provision of such a method, and the apparatus therefor, practiced so that the metal introduced into the mold is uniformly distributed in a very short time without material internal disturbance while the metal is in a free flowing condition and is rapidly brought to a quiescent state as soon as the even distribution is obtained; the still further provision of a method of preparing a refractory mold so that the molten metal will flow in the mold without that detrimental disturbance accompanying prior methods of this kind; the further provision of a mold and the method of preparing the same with a facing so as to produce a membranous or shell-like coating performing such functions as conditioning the surface of the sand to enable it to withstand the cutting action of the metal, of making the mold wall smooth and impervious to the flowing iron, of resisting the washing effect of the iron, and of being of such a nature as to fuse to the skin of the casting to supply the same with a protective surface coating. Still further and correlated objects of the invention include the process of producing the hollow bodies with the protective coating or facing and the product so obtained; and the provision of a refractory mold having a sand composition which obviates the mechanical drawbacks found in prior practice and which permits of obtaining non-defective and clean castings.

To the accomplishment of the foregoing and such other objects as may hereinafter appear, my invention consists in the methods, the steps and the elements and their relation one to the other, as hereinafter particularly described and sought to be defined in the claims, reference being had to the accompanying drawings which show a preferred embodiment of my invention, and in which:

Fig. 1 is an elevational view of my casting apparatus showing the same in one stage of operation,

Fig. 2 is a plan view of the same,

Fig. 3 is an elevational view taken in cross-section on the line 3—3, Fig. 1,

Fig. 4 is an elevational view taken in cross-section on the line 4—4, Fig. 1, showing the machine in another stage of operation,

Fig. 5 is a view taken in cross-section on line 5—5, Fig. 1, and showing the manner of removing a filled mold and substituting an unfilled mold therefor,

Fig. 6 is a view of the mold showing the details thereof and the manner of producing the sand lining therein.

Fig. 7 is a cross-sectional detail view of the mold showing a pipe casting therein,

Fig. 8 is a detail view showing the preferred construction of the means for charging the mold,

Fig. 9 is a view taken in cross-section on the line 9—9, Fig. 8, and

Fig. 10 is a cross-sectional view of the mold taken in the line 10—10, Fig. 7.

10 As heretofore mentioned, a principal desideratum of this invention centers about the provision of a process for centrifugally casting on refractory such as "green" sand molds in which the molten metal is so introduced into the mold and the mold so coordinateley operated as to effect a uniform distribution of the molten metal to produce a uniform and homogeneous casting product. It has been previously well known 20 that the temperature conditions of the mold and molten metal at the time of charging the mold and the time factor involved in charging were highly important considerations in producing uniform metal distribution. Intimately interrelated with the temperature and time factors is also that of the kinetic behaviour or action of the fluid metal in the mold having components due not only to the centrifugal action of the 25 mold, but to the head of the metal when introduced into the mold and the reflecting action of the mold ends which produces a surging of the liquid metal mass back and forth from end to end of the mold. After 30 considerable experimentation, I have found that these temperature, time and energy factors may be controlled so as to permit of producing commercial pipe in a satisfactory manner.

40 I have discovered after extensive research that the molten metal should preferably be introduced into the mold at certain temperatures between predetermined high and low values in the quickest possible time, and that 45 the mold should preferably be so operated and manipulated as to substantially inhibit the disturbance incident to and resulting from the introduction of the metal in this manner, to minimize the splashing and 50 surging effect and to bring the same to a quiescent state rapidly and before congealing temperatures have been reached. More specifically, I have empirically determined that the best results can be obtained by 55 delivering the whole charge of molten metal into the rotating mold, preferably at one end thereof, in the shortest possible time, with the molten metal at temperatures hereinafter more fully described, and that to 60 rapidly eliminate the surging and to produce a quiescent mass and obtain an even distribution, the mold should preferably be supported in a position inclined to the horizontal during discharge or delivery of the 65 metal thereto, and should then be moved

quickly and quietly to horizontal position while the metal is still in a fluid or free flowing state.

By inclining the mold at the proper angle with reference to the horizontal plane, the metal can be introduced into the flask or mold in the quickest possible period either with the mold revolving or stationary, and at the same time the metal may be caused to arrive at the far or lower end of the mold 70 with a minimum amount of surge which almost immediately quiets itself, after which when the mold is lowered the metal quietly distributes itself uniformly over the mold surface from end to end and without leaving any trace of surge in the casting.

Referring now to the drawings, in which I show a centrifugal casting machine embodying the principles of my invention and which now forms in practice a preferred embodiment of the apparatus employed in carrying out the process, and referring more particularly to Figs. 1 to 5, I provide a rotary mold comprising a flask 10 having a plurality of perforations 11 distributed over the body of the same and forming vent holes for the gases and steam generated during a casting operation, the said flask 10 being provided with a refractory lining such as the sand lining 12 (see for example Figs. 3 to 5), which lining is preferably surfaced with a facing 13. The mold is mounted and arranged for movement between a horizontal position and a position inclined to the horizontal, the latter position being indicated in Fig. 1 of the drawings, and to this end the mold is mounted on a supporting structure 14 which is arranged for corresponding movement between horizontal and inclined positions, a desirable construction 105 including the mounting of the frame 14 for movement about a horizontal axis provided by the spaced standards 15, 15 in which the frame 14 is journaled for the desired motion, as will clearly appear from a consideration of the drawings.

Any suitable mechanism may be employed for moving the mold and its supporting frame between the horizontal and inclined positions. In the illustrated mechanism there is preferably provided a cross shaft 16 journaled in the spaced uprights 17, 17, which shaft receives motion from a longitudinally arranged drive shaft 18 by means of a worm 19 fixed on the drive shaft 18 and a worm wheel 20 meshing therewith and fixed on the cross shaft 16, the cross shaft being provided with the spaced eccentrics 20', 20' embraced by the eccentric straps 21, 21, which latter are dependingly carried by the frame 14, the eccentric straps being to this end provided with terminal forks 22, 22 pivotally mounted in the depending bearing lugs 23, 23 formed with the frame 14. With this construction it will be seen that upon rotation 120

tion of the cross shaft 16 the desired motion will be imparted to the frame 14 and the mold supported thereby. For controlling the movement of the mold from the drive shaft 18, I may provide the clutch mechanism of any approved type such as indicated at 24, the clutch mechanism being controlled by means of the clutch lever 25.

Also for the purpose of definitely limiting the movement of the frame 14 in the horizontal position, I may provide stop means which in the preferred construction includes the adjustable bolts 26, 26 carried by the standards 17, 17 against which the stop lugs 27, 27 carried by the frame 14 are adapted to abut. A comparison of Fig. 1 and Fig. 4 will indicate the association of the parts of the apparatus when the mold assumes the inclined position and the horizontal position, Fig. 1 indicating the frame 14 at a position near the maximum or high point of the cam or eccentric 20', and Fig. 4 indicating the frame in its lowermost horizontal position with the stop lugs 27 abutting the bolts 26.

To prevent any surging of the metal when the same is introduced into the mold, and to aid in bringing about stabilizing conditions of the mold, preferably only the pouring end of the same is open, and the lower end of the same is preferably completely or substantially completely closed. Referring now to Figs. 6, 7 and 8 of the drawings, the open or pouring end of the mold is shown to comprise an annular flange 28 which is screwed onto and made part of the flask 10, and to which is bolted a stripper plate 29 by means of two countersunk key bolts 29', a stop-off plate 30 being provided and bolted to the stripper plate 29 by means of the two countersunk key bolts 31. The stop-off plate 30 is flanged in opposite directions to provide the tubular structure shown at 31', and with this construction the plate may be reversed from time to time, thus prolonging its life. The inner diameter of this tubular structure 31' is so predetermined as to be somewhat less than the inner diameter of the pipe to be formed, as will be readily understood by those skilled in the art. The other end of the flask 10 may be provided with the bell mouth structure 32, to which is bolted the end plate 33 provided with a substantially completely closed core 34 which in some instances may be provided with a suitable vent opening as shown in dotted lines in Fig. 7 of the drawings. The core 34 may be carried by the end plate 33 by means of the wedge keys 34', the core having the configuration for forming the inner surface of the bell mouth end of the pipe, as is clearly shown in Fig. 7 of the drawings, the outer configuration of the pipe being determined by that of the sand lining at the bell mouth end, as will be readily understood by

those skilled in the art. With this arrangement the stop-off plate, the stripper plate and the end plate 33 may be readily removed to permit the removal of the sand and the casting after a casting operation has been performed. By completely or substantially closing the end of the mold, the metal may be poured into the mold when inclined without causing a surging of the metal, the substantially closed end also aiding in stabilizing pressure conditions in the mold.

In the practice of the method as will presently appear, a "poured" mold is removed from the casting machine and is replaced by a fresh or "unpoured" mold, and to this end the flask 10 is removably mounted on the supporting structure 14. Referring for example to Figs. 1 to 4 of the drawings, I show the flask arranged for rotary motion on spaced sets of rollers. One set of rollers, as for example the rear set, comprises the rollers 35, 35 journaled on a bracketed structure 36 fixedly carried by the frame 14 and a roller 37 carried by a yoke 38 which is pivoted at one end 39 on the frame 14 and movably secured at its other end 40 by means of the bolt locking member 41 and the spring 42, the latter being provided as a vibration-absorbing means and as a means for permitting circumferential expansion of the flask when heated by the molten metal. The other set of rollers also comprises two spaced rollers 43 journaled in a bracketed structure 44 fixedly carried by the frame 14 and a roller 45 journaled in a yoke 46 which is also pivotally mounted as at 47 and movably locked in position by means of the locking elements generally designated as 48, and similar in structure to that above described. The flask 10 is preferably provided with the spaced bands 49 and 50, the band 49 being preferably grooved to receive the rollers 35 and 37, which are convexed, and the band 50 being preferably straight faced to receive the correspondingly contoured rollers 43 and 45, this latter construction being provided to permit axial expansion of the flask when heated.

When it is desired to remove a mold after casting and replace the same by a freshly prepared mold, the yokes 38 and 46 are unlocked and moved to open position as will be readily understood, and the filled flask is then removed. For removing the flask I provide any suitable elevating means which in the construction shown comprises the elevating rails 51, 51 shown particularly in Figs. 1, 2 and 5, the said rails being journaled at one end on the spaced standards 52, 52 located adjacent the rolling stock 53 over which wheeled trucks 54 are adapted to move, and the other end of each of the rails 51 being provided with a curved section 55 adapted to engage the flask 10 and

elevate the same from the full line position shown in Fig. 5 to the dotted line position shown for clearing the lower roller sets 35 and 43 respectively. From a consideration of Fig. 5, it will be seen that the rails 51 are arranged to assume a horizontal position when the flask is elevated so that the flask may with facility be conveyed to the wheeled truck 54 and so that a newly prepared flask may be conveyed with equal facility from the truck to the casting machine.

For elevating and lowering the rails 51 any suitable mechanical means may be employed. I preferably provide a vertically movable screw rod 56 connected to a cross-tie rail 57 uniting the rails 51, the said screw rod being caused to elevate or descend by means of the worm wheel 58 journalled for rotation in a casing 59 and engaging the thread 60 of the screw rod, the said worm wheel being adapted to be driven in either direction by means of a worm 61 fixed on the drive shaft 18, a clutch mechanism 62 of any approved type being provided to control the operation of the elevating mechanism.

For rotating the mold I preferably provide a driving means which is directly connected to the flask 10 and is arranged to permit rapid removal of a filled mold after a casting operation. In the preferred construction I provide a motor 63 whose axis is alined with the axis of the rotary mold, the said motor being directly connected to the mold by a quickly detachable connection comprising a coupler 64 provided with a drive key 65 loosely received in grooves 66 in the end plate 33, the said motor being mounted for axial motion in the guides 67 to cause the engagement and disengagement of the driving key with the flask, the motor being moved by means of a threaded rod 68 actuated by a hand wheel 69. Preferably the driving connection between the coupler 64 and the end plate 33 is a resilient or flexible one, and to this end the key 65 is attached to a metal reinforced fabric disk 64<sup>a</sup> which is carried by and bolted to the coupler 64. With this construction it will be seen that not only will the mold be driven with a minimum of vibration, but that the mold may be quickly coupled and uncoupled from the driving means to effect rapid interchangeability of the molds. It will be further seen that by providing the motor and the flask at opposite sides of the axis of the supporting frame 14, that a desirable balanced construction is obtained.

For charging the mold with molten metal I may provide the runner box 70 carried by the wheeled truck 71 which may be carried by the frame 14 as shown, the said runner box being provided with a pouring spout 72 which may project a short distance into the

open end of the flask 10. While the runner box is shown mounted on the frame 14, it will be understood that it may desirably be mounted independent of the machine itself so as to reduce the weight carried by the frame and produce a more balanced construction.

It will be noted that in the operation of my casting machine the uniform distribution of the metal over the entire mold is obtained in a simple manner by pouring the metal at one end thereof, the desired distribution being obtained without the use of the complicated mechanism heretofore found necessary in casting hollow bodies in elongated molds such as dumping troughs and pouring spouts which are caused to move longitudinally of the mold.

In operating the casting machine described, the time factor, the inclination of the machine and the manner of manipulating the same are important considerations. I have found experimentally that the best results can be obtained by delivering the whole charge of molten metal into the mold in the quickest possible time, say for instance about three seconds in the case of pipes of about six inches in diameter. In order to obtain the even distribution of the metal throughout the mold from end to end, including the bell mouth as well as the spigot, I have found an incline of the mold of  $\frac{1}{2}$  inch to the foot to yield very satisfactory results, but the degree of inclination will vary somewhat depending upon the diameter and length of the pipe being cast. By inclining the mold moreover so that the metal flows towards the bell end, I find that the metal is quickly supplied in the desired quantities to form the bell end in an efficient manner.

In operating, the metal is poured from one end into the mold opening and towards the bell mouth, and immediately the full charge in bulk is delivered into the mold or in fact in some instances before the entire charge has been completely dumped into the mold, I begin to lower the mold from its inclined to its horizontal position; and this lowering should be gradual and quiet so as not to create too much disturbance of the molten metal and at the same time should be accomplished quickly, as for example in three or more seconds depending upon the size and length of the pipe being cast, speed being desirable if not indeed essential to the whole process. If this lowering of the mold is not done quickly and while the metal is in a free flowing condition, the distribution of the metal endwise is not uniform. This action will be readily understood when it is seen that the bulk of the charge of metal originally introduced flows to the lower or bell mouth end of the mold, and as the mold is lowered into a horizontal position this

metal flows back towards the spigot end and in doing so is picked up and uniformly disposed on the mold surface. Now it is readily understood that at a given number of revolutions of the mold per minute, the mold will only carry a definite amount of iron on its surface, so that any additional iron in the fluid state will pass by until it reaches a point which is not already carrying the proper amount of metal, and that if this metal has assumed a congealing or pasty state, then the carrying capacity of the mold for the metal is substantially increased, and instead of allowing the metal to flow back to the spigot end, it is picked up and held on the surface of the mold with the result that an uneven pipe endwise is produced. This carrying capacity of the mold face changes with the change in the fluidity in the metal, so that it is highly desirable that the whole operation be accomplished and the horizontal position be attained while the metal is still in a thoroughly fluid state, so that it can dispose itself uniformly over the mold surface.

The temperature conditions of the mold and the metal as already briefly mentioned are important considerations. If the metal is poured cold or below certain temperatures, the portions picked up by the mold surface as the metal flows to the bell end sets up or becomes gummy too rapidly, and before the metal moving from the bell end towards the spigot end returns to it, thereby preventing a proper uniting of the metal and forming a lap or fold. If on the other hand the metal is at too high a temperature, as for example much more than 2400° F., say approaching 2500° F., the metal is in too fluid a condition and too unstable, and has a tendency to cause a wave or splash which does not readily lose itself or spend itself before the setting action takes place. I have therefore found that the temperature of the molten metal should be about 2300° F. or higher, and preferably below the maximum limit noted. The temperatures I preferably employ are based on the freezing point of the iron between 2000° F. and 2050° F., and it will be therefore understood that since the freezing point of the metal is a variable depending on the alloys or elements mixed therewith, as for example the carbon content of the same, that the working temperatures may be varied within the principles herein set forth.

The metal pouring operation is approximately as follows:

understood by those skilled in the art, of 65 a measuring ladle, and this ladle is taken to the furnace and filled with a definite amount of iron sufficient for the making of one pipe. The ladle is then conducted to the casting machine, and the time of conveyance should not consume more than 30 to 60 seconds. The casting machine having previously been elevated to the proper angle to the horizontal, the mold is set in motion to spin at the proper speed, with the casting spout or runner in position projecting slightly into the spigot end of the mold. The ladle of iron coming from the furnace is immediately dumped, or poured, into the runner, and this operation should consume 75 from about 3 to 5 seconds. Immediately following this step, if not overlapping the same, the operation of moving the machine from its inclined position to the horizontal 80 position is begun, and is accomplished in 85 from 2 to 5 seconds, so that the entire operation of casting from the time the metal comes to the proper pouring temperature until the mold has assumed a horizontal 90 position should preferably not exceed one 95 minute and ten seconds, and less if possible, a desideratum being the provision of the maximum length of time from the time the mold comes to a horizontal position until the iron passes from the fluid state to a semi-fluid or gummy state, at which time it will cease to distribute itself over the 100 face of the mold. The pouring operation having been completed and the mold brought back to the horizontal position, it is desirable to continue spinning the mold at or near full speed for say about a minute, at which time the metal has taken its initial set, and the casting speed of the mold can then be reduced to about half its original speed and continue to spin for a period of about 2 to 3 minutes more or less depending upon the size of the pipe being cast, at which time the spinning operation 105 is discontinued and the flask with the sand and the pipe contained in the same is removed from the machine to be substituted by another freshly prepared mold.

The molten iron from the moment it begins to run from the furnace burns from contact with the air, and the oxidation continues as long as the iron is exposed to the air. The oxide produced unites with any silicious material available to form a slight slag which floats on the surface. When the metal is dumped into the runner and into the mold, a small amount of this slag

near the bell end, whence it can be easily removed by a grinding or scouring operation. It is desirable to further localize this slag, and to this end I may, prior to 5 lowering the mold from its inclined position, impart to the mold a sudden and short upward "kick" to cause the dross to collect or localize at the bell end of the mold for easy removal therefrom. To accomplish 10 these ends the frame 14 when elevated for a pouring operation is positioned so that the highest points of the eccentrics 20', 20' are slightly in advance of the maximum elevating position, this so that after or over 15 lapping the pouring step the eccentrics 20', 20' when rotated are first rotated to the high points thereof and then beyond, so that a short elevating "kick" is produced prior to the lowering step.

20 For the purpose of permitting a free and undisturbed flow of metal from the pouring spout into the mold, and to the end of aiding in stabilizing the conditions in the mold, liberal provision is made to allow the free 25 passage of gas out of the mold while the iron is being introduced therein. The desirability of making such provision will be readily seen when it is understood that the 30 volume of air in the mold when subjected to the temperature of the hot iron introduced therein changes very rapidly and to about five times the original value, and unless provision is made for these gases to free 35 themselves from the mold, undesirable pressure is immediately created within the mold which may cause a blow through whatever 40 openings are available, and on certain occasions when the pouring opening of the mold is sufficiently restricted, may tend to blow the iron back through the pouring spout. To 45 obviate this undesirable behaviour, the pouring spout projecting into the mold is constructed so as to cover a portion only of the mold opening, and is arranged to permit 50 another portion of the opening to remain unobstructed for the free egress of hot gases from the mold. This is shown particularly in Figs. 8 and 9 of the drawings, and referring to these figures, the 55 pouring spout 72 heretofore mentioned is constructed so as to occupy a portion only of the flask opening and preferably the lower half of the flask, leaving another portion and preferably the upper half of the opening 60 unobstructed for permitting a free egress of the gases from the mold. As shown the spout 72, which is preferably but not necessarily made of a composition of graphite similar to that used for furnace electrodes, is semi-circular in cross-section and is arranged as close as possible to the walls of the flask opening to prevent any passage of 65 gas and iron at the lower half of the same. Also preferably I provide attached to the pouring spout or the runner a metal shield

73 for protecting the operator from the heated gas coming from the mold.

As hereinbefore briefly stated, another important object of this invention relates to the production of a refractory mold of a 70 character and composition to obviate the mechanical objections found in prior practice, to permit of obtaining non-defective castings, and to permit the molten metal to flow over the mold surface without setting 75 up the disturbances hitherto encountered. As mentioned, the refractory lining which I prefer to employ in the mold consists of a sand mixture and more particularly a "green" or unbaked sand. I have found that the moisture content of the sand mixture plays a highly important rôle in the production of a meritorious casting, the sand if in 80 too dry a state having the objection of not possessing bonding power sufficient to support itself to withstand the cutting and washing action of the iron and the centrifugal action of the mold, and if in too moist a state giving rise to too copious a generation 85 of steam and gas more than the sand is capable of taking care of, with the result that the steam is blown into the metal instead of out through the mold, making a honeycomb or pocketed casting. I have discovered that with a predetermined moisture content in the sand mixture and further with 90 certain constituents therein, the sand may be made of the desired consistency and character to avoid on the one hand the mechanical difficulties, and the washing of the fluid metal, and to obviate on the other hand the objectionable degree of generation 95 of steam. I have further discovered that in order to properly handle iron on a "green" sand mold so that the metal flows therein without material disturbance, that the manner of ramming the mold is of great importance, it being highly desirable that the 100 mold be rammed of uniform density.

To produce a mold having these desired characteristics, I first preferably prepare a sand mixture described and claimed in my copending application Ser. No. 623,650 filed March 8, 1923, having the composition hereinbelow referred to, the sand mixture possessing a moisture content of from 7% to 11% calculated on the weight of the dry sand and the flask is lined with this sand mixture and rammed by means of a jolt 105 rammer.

For the sand lining, I preferably employ a mixture of silica sand, molding sand and sharp sand containing from 7% to 11% moisture, and I have found the following 115 mixture to give very desirable results:

|              | Per cent. |
|--------------|-----------|
| Silica sand  | 50        |
| Sharp sand   | 35        |
| Molding sand | 15        |

The rational analysis of this sand is found to be as follows:

|                  | Per cent. |
|------------------|-----------|
| Quartz           | 80 to 85  |
| Clay             | 5 to 10   |
| Feldspar         | 5 to 10   |
| Uncombined water | 7 to 11   |

This sand mixture is then rammed in the flask by means of a jolt rammer which is operated either with air or electricity. This step is carried out by placing the flask on a jolt rammer in a vertical position by inserting a head pattern 74 (Fig. 6) at the bell end thereof and by inserting a pattern 75 therein, and by then introducing the sand into the mold, the ramming operation proceeding either after completely filling up the flask or as the sand is being introduced. I have found that by the jolt ramming of "green" sand, the density of the sand at any area is consistent or uniform, and that although the density may change from one end of the flask to the other, it changes uniformly from a heavy density at the lower end of the flask to a light density at the upper end of the flask, with a uniform variation along the length of the mold, eliminating alternate hard and soft spots which in practice has been demonstrated to be highly objectionable, alternate hard and soft areas such as produced for example by hand ramming or pneumatic ramming being one of the chief causes of internal disturbance in the flowing metal which are detrimental to a proper casting operation.

The provision of a facing for the refractory lining which satisfactorily withstands destruction when the metal is poured, and which is so associated with the lining as to aid in preventing the breaking and cutting of the same by the molten metal I have found to be of the utmost importance in a centrifugal refractory mold, and forms, as already briefly mentioned, another prime object of my invention.

In the prior art numerous facings of sand molds to permit the clean cleaving of the casting from the sand and the obtaining of castings of the desired hue have been suggested and used, the facings including powdered, liquid or plastic substances such as plumbago, carbon, clay, etc., applied to the inner surface of the lining. The use of these facings, has, however, been found unsatisfactory in centrifugal casting operations. By my present invention I propose to employ a facing material which is applied to the surface of the "green" sand mold in a powdered state, the powdered material having the properties of absorbing moisture from the sand lining, of taking a quick initial set to produce a membranous or skin-like mold facing which is highly refractory, of having a low capacity for ab-

sorption of heat, and of producing mold walls impervious to the molten metal. I have discovered that such a facing may be produced with the use of natural cement, this being a pulverized product resulting from the calcination of an argillaceous limestone at a temperature only sufficient to drive off the carbon dioxide.

The powdered natural cement may be applied to the face of the "green" sand mold by means of the apparatus disclosed and claimed in my copending application Ser. No. 587,999 filed Sept. 13, 1922, for a mold facing device, the result obtained being generally indicated in Figs. 3 to 5 for example, the facing 13 representing the membranous cement casting obtained.

Immediately the application is made, the powdered cement begins to absorb moisture from the sand and chemically reacts to quickly take an initial set, producing instead of a soft powdered face a rather shell-like or skin-like face which displays a high resistance to the cutting action of the iron. Highly advantageous properties of my cement facing are the quick set that takes place without the application of heat and the fact that the natural cement in contradistinction from other facings and even other cements which on setting contract and pull away from the surface of the sand, expands on setting with the result that the facing tends to pack itself or imbed itself into the sand mold proper and in the grains of the sand on the face of the mold so as to become practically an integral part thereof, the effect including a conditioning of the sand lining for the high resistance to destruction displayed thereby when the metal is poured thereon.

Another important property of my cement facing is its neutral or basic character so that no chemical reaction is set up between the iron oxide on the surface and the material of which the facing is composed. With the natural cement facing employed, the sand is protected from the iron oxide and when the casting is made the same may be separated with ease from the sand.

While in most instance I may employ natural cement in its natural state, in some instances I prefer to mix with the natural cement a small percentage, say from 5 to 10%, of an unctuous material such as graphite or talc, the purpose of this being to act as a lubricant to aid in the spreading of the powdered cement on the face of the mold. Also in some instances where a comparatively thick facing body or wall is desired to be produced, I may impregnate the exposed surface of the cement facing with moisture as by means of a spray or atomizer, causing the cement facing to take a quick initial set throughout the body thereof.

By coating the surface of the mold with the natural cement facing, I have found

that in addition to providing the facing having the characteristics above mentioned, I am enabled to produce a casting product having a facing or coating which forms a protection against corrosive and other deteriorating action. The membranous facing produced on the sand lining is of a fusible character and is fused by contact with the molten iron after the metal is poured, the fusion resulting in the pipe retaining a large portion of the cement which forms a coating or lining on its outer surface or skin, such as indicated at 76 in Fig. 7 of the drawings. It is well known that cement inhibits corrosion in all iron products, and the fusing of the iron with the cement therefore produces a protective and highly desirable coating. While the cement is fused, it is to be noted that due to the highly non-conducting character of the cement the sand does not attain sufficient temperature to fuse with the cement and the cement coated casting is produced in a smooth and clean condition.

25 The practice of my method and the operation of the apparatus will in the main be fully apparent from the above detailed description thereof. It will be further understood by those skilled in the art to which this invention appertains that with the use of my process, centrifugally cast bodies and especially ferrous pipe may be made with great economy to produce pipe having not only that increased tensile strength, 35 modulus of elasticity and modulus of rupture characteristic of centrifugally produced metal products, but the strong and annealed, easily machinable properties of cast iron together with the high resistance to 40 the corrosive influences met with under actual service conditions. It will be further seen that the apparatus employed is inexpensive and durable, and may be operated with ease and facility. It will be further 45 seen that the mold may be charged in a simple manner, the pouring of the metal and the operation of the mold following simple laws, permitting the employment of labor not necessarily skilled. With my process, 50 furthermore, I have found that a cheap metal mixture may be employed, such for example as a metal mixture having the elements phosphorus, carbon, silicon, manganese and sulphur, reduced to as low as 5%, 55 and the silicon content reduced from about 11% down to  $\frac{1}{16}\%$ , this being materially lower than the costly silicon content employed in mixtures with other processes. It will therefore be seen that the practice of the 60 method is generally characterized by the ease of practicing the process, the small cost of the apparatus and its upkeep, the efficient product, and the inexpensive metal mixture employed.

65 It will be understood that while I have

described my invention in great detail so that anyone skilled in the art may be enabled to practice the same, that I do not intend to be limited to the details either in the process or in the apparatus employed, 70 and that some of the improvements either in the process or in the machine may be used without some of the other improvements described, the intent of the above detailed description being to exemplify the manner 75 in which the numerous problems involved may be successfully solved, all the examples being given by way of illustration only, and not by way of limitation. It will be further clear that numerous changes may be 80 made without departing from the spirit of the invention defined in the claims hereto appended, and in other claims to the subject-matter herein disclosed and set forth in other of my copending applications 85 centrifugal refractory mold and method of preparing the same, Serial No. 623,748, filed March 8, 1923; art of producing centrifugal castings with a protective coating, Serial No. 623,649, filed March 8, 1923, and composition of matter for molds, Serial No. 623,650, filed March 8, 1923.

1 claim—

1. In the art of centrifugally casting hollow metal bodies, the method which consists in pouring molten metal into a rotary mold while the latter is in a position inclined to the horizontal, and in moving the mold to a substantially horizontal position while the metal is still in a fluid condition. 100

2. In the art of centrifugally casting hollow metal bodies the method which consists in discharging molten metal in bulk for delivery into a rotary mold while the latter is in a position inclined to the horizontal, and in moving the mold to a substantially horizontal position while the metal is still in a fluid condition. 105

3. In the art of centrifugally casting hollow metal bodies, the method which consists in charging a rotary mold with molten metal having a predetermined temperature while the mold is in a position inclined to the horizontal, and in moving the mold to a substantially level or horizontal position while the metal is still in a fluid condition, the temperature being so predetermined as to permit the metal to remain in a fluid or free flowing state during the time of charging and time of levelling of the mold. 110

4. In the art of centrifugally casting hollow metal bodies, the method which consists in charging a rotary mold with molten metal at a predetermined temperature while the mold is in a position inclined to the horizontal, and in moving the mold to a substantially level or horizontal position while the metal is still in a fluid condition, the temperature being so predetermined as to permit the metal to remain in a fluid or free 115 120 125 130

flowing state during the time of charging and time of levelling of the mold and to then assume a congealing state.

5. In the art of centrifugally casting hollow metal bodies, the method which consists in tilting a rotary mold to a position inclined to the horizontal, in pouring molten metal into the mold at the elevated end thereof, and in moving the mold to a substantially horizontal position while the metal is still in a fluid condition.

6. In the art of centrifugally casting hollow metal bodies, the method which consists in tilting a rotary mold to a position inclined to the horizontal, in discharging molten metal in bulk into the mold at the elevated end thereof, and in moving the rotary mold to a substantially horizontal position while the metal is still in a fluid state.

20 7. In the method of centrifugally casting hollow metal bodies, the steps which consist in introducing molten metal into one end of a rotary mold while the latter is in a position inclined to the horizontal, and in immediately lowering the mold to a substantially horizontal position.

30 8. In the art of centrifugally casting hollow metal bodies the method which consists in providing a rotary mold substantially closed at one end and tilting the same in a position inclined to the horizontal, in discharging molten metal into the mold at the other end thereof, and in moving the mold to a substantially horizontal position while the metal is still in a fluid condition.

40 9. In the art of centrifugally casting hollow metal bodies, the method which consists in pouring molten metal into a rotary refractory mold while the latter is in a position inclined to the horizontal, and in moving the rotary mold to a substantially horizontal position while the metal is still in a fluid condition.

45 10. In the art of centrifugally casting hollow metal bodies, the method which consists in pouring molten metal into a rotary green sand mold while the latter is in a position inclined to the horizontal, and in moving the rotary mold to a substantially horizontal position while the metal is still in a fluid condition.

55 11. In the art of centrifugally casting hollow metal bodies, the method which consists in pouring molten metal into a rotary refractory mold provided with a membranous facing expanded onto the inner wall of the same, while the mold is in a position inclined to the horizontal, and in moving the mold to a substantially horizontal position while the metal is still in a fluid condition.

60 12. In the art of centrifugally casting hollow metal bodies, the method which consists in pouring molten metal into a rotary refractory mold provided with a cement

facing, while the mold is in a position inclined to the horizontal, and in moving the mold to a substantially horizontal position while the metal is still in a fluid condition.

70 13. In the art of centrifugally casting hollow metal bodies, the method which consists in pouring molten metal into a rotary mold made of refractory material having a moisture content of not less than 7% while the mold is in a position inclined to the horizontal, and in moving the mold to a substantially horizontal position while the metal is still in a fluid condition.

75 14. In the art of centrifugally casting hollow metal bodies, the method which consists in pouring molten metal into a rotary mold made of refractory material having a moisture content not more than 11% while the mold is in a position inclined to the horizontal, and in moving the mold to a substantially horizontal position while the metal is still in a fluid condition.

80 15. In the art of centrifugally casting hollow metal bodies, the method which consists in pouring molten metal into a rotary mold made of refractory material having a moisture content of from 7 to 11% while the mold is in a position inclined to the horizontal, and in moving the mold to a substantially horizontal position while the metal is still in a fluid condition.

85 16. In the art of centrifugally casting hollow metal bodies, the method which consists in pouring molten metal into a rotary mold made of refractory material having a moisture content of from 7 to 11% and provided with a cement facing, while the mold is in a position inclined to the horizontal, and in moving the mold to a substantially horizontal position while the metal is still in a fluid condition.

90 17. In the art of centrifugally casting hollow metal bodies, the method of localizing the dross which consists in pouring molten metal into a rotary mold while the latter is in a position inclined to the horizontal, and in imparting to the mold first an elevating movement to increase the inclination, and then a lowering movement to substantially horizontal position while the metal is still in a fluid condition.

100 18. In the art of centrifugally casting hollow metal bodies, the method of localizing the dross which consists in pouring molten metal into a rotary mold while the latter is in a position inclined to the horizontal, and in imparting to the mold first a sharp and short elevating movement to increase the inclination, and then a gradual lowering movement to substantially horizontal position while the metal is still in a fluid condition.

110 19. In the art of centrifugally casting hollow metal bodies, the method which consists in coating a green sand mold with

a membranous facing, in pouring molten metal into the mold while the latter is in a position inclined to the horizontal, and in moving the mold to a substantially horizontal position while the metal is still in a fluid state.

20. An apparatus for centrifugally casting hollow metal bodies comprising a rotary mold mounted for movement between a substantially horizontal position and a position inclined to the horizontal, means for charging molten metal into the mold when the latter is in the inclined position, and provisions for rapidly moving the mold to the horizontal position while the metal is still in a fluid condition.

21. An apparatus for centrifugally casting hollow metal bodies comprising a rotary mold mounted for movement between a substantially horizontal position and a position inclined to the horizontal, means for charging molten metal into one end of the mold when the latter is in the inclined position, and provisions for quickly moving the mold to the horizontal position while the metal is still in a fluid condition.

22. An apparatus for centrifugally casting hollow metal bodies comprising a rotary mold substantially closed at one end and open at the other end, the said mold being mounted for movement between a substantially horizontal position and a position inclined to the horizontal, means for charging molten metal into the open end of the mold with the latter in the inclined position, and provisions for moving the mold to the horizontal position while the metal is still in the fluid condition.

23. An apparatus for centrifugally casting hollow metal bodies comprising a rotary refractory mold mounted for movement between a substantially horizontal position and a position inclined to the horizontal, means for charging molten metal into the mold when the latter is in the inclined position, and provisions for rapidly moving the mold to the horizontal position while the metal is still in a fluid state.

24. An apparatus for centrifugally casting hollow metal bodies comprising a rotary green sand mold mounted for movement between a substantially horizontal position and a position inclined to the horizontal, means for charging molten metal into the mold when the latter is in the inclined position, and provisions for moving the mold to the horizontal position while the metal is still in a fluid condition.

25. An apparatus for centrifugally casting hollow metal bodies comprising a rotary refractory mold provided with a membranous facing expanded onto the inner wall of the same, the said mold being mounted for movement between a substantially horizontal position and a position inclined to the

horizontal, means for charging molten metal into the mold when the latter is in the inclined position, and provisions for moving the mold to the horizontal position while the metal is still in a fluid condition.

26. An apparatus for centrifugally casting hollow metal bodies comprising a rotary refractory mold provided with a membranous and fusible facing expanded onto the inner wall of the same, the said mold being mounted for movement between a substantially horizontal position and a position inclined to the horizontal, means for charging molten metal into the mold when the latter is in the inclined position, and provisions for moving the mold to the horizontal position while the metal is still in a fluid condition.

27. An apparatus for centrifugally casting hollow metal bodies comprising a rotary refractory mold provided with a cement facing, the said mold being mounted for movement between a substantially horizontal position and a position inclined to the horizontal, means for charging molten metal into the mold when the latter is in the inclined position, and provisions for moving the mold to the horizontal position while the metal is still in a fluid condition.

28. An apparatus for centrifugally casting hollow metal bodies comprising a rotary mold made of a refractory material having a moisture content of from 7 to 11%, said mold being mounted for movement between a substantially horizontal position and a position inclined to the horizontal, means for charging molten metal into the mold when the latter is in the inclined position, and provisions for moving the mold to the horizontal position while the metal is still in a fluid condition.

29. An apparatus for centrifugally casting hollow metal bodies comprising a rotary mold made of a refractory material having a moisture content of 7 to 11% and provided with a cement facing, the said mold being mounted for movement between a substantially horizontal position and a position inclined to the horizontal, means for charging molten metal into the mold when the latter is in the inclined position, and provisions for moving the mold to the horizontal position while the metal is still in a fluid condition.

30. An apparatus for centrifugally casting hollow metal bodies comprising a rotary green sand mold provided with a cement facing, the said mold being substantially closed at one end and open at the other end and being mounted for movement between a horizontal position and a position inclined to the horizontal, means for charging molten metal into the open end of the mold while the latter is in the inclined position, and provisions for moving the mold to the horizontal position while the metal is still in a fluid condition.

horizontal position when the metal is still in a fluid condition.

31. An apparatus for centrifugally casting hollow metal bodies comprising a rotary mold mounted for movement between a substantially horizontal position and an elevated position inclined to the horizontal, means for charging molten metal into the mold when the latter is in the inclined position, and provisions for first imparting a quick further elevating movement to the mold and for then lowering the same to the horizontal position while the metal is still in a fluid condition.
32. An apparatus for centrifugally casting hollow metal bodies comprising a rotary mold, means for supporting the same for movement about an axis adjacent one end thereof, and provisions for moving the same about said axis.

33. An apparatus for centrifugally casting hollow metal bodies comprising a rotary mold, means for supporting the same for movement about a horizontal axis adjacent one end thereof, and provisions adjacent the other end thereof for moving the same about said axis.

34. An apparatus for centrifugally casting hollow metal bodies comprising a rotary mold, a supporting frame therefor, the said supporting frame being mounted for pivotal motion about an axis adjacent one end of the mold, and provisions for moving the supporting frame about the said axis to elevate and lower the mold.

35. An apparatus for centrifugally casting hollow metal bodies comprising a rotary mold, a supporting frame therefor, the said supporting frame being mounted for pivotal motion about an axis adjacent one end of the mold, and provisions adjacent the other end of the mold for moving the supporting frame about the said axis to elevate and lower the mold.

36. An apparatus for centrifugally casting hollow metal bodies comprising a rotary mold, a supporting frame therefor, the said supporting frame being mounted for pivotal motion about an axis adjacent one end of the mold, means supported by said frame and arranged on one side of said axis for rotating the mold, and provisions arranged on the other side of said axis for moving the frame to elevate and lower the mold.

37. An apparatus for centrifugally casting hollow metal bodies comprising a rotary mold, means for supporting the same for movement about an axis adjacent one end thereof, means adjacent the other end thereof for charging the mold with molten metal, and provisions for moving the mold about said axis.

38. An apparatus for centrifugally casting hollow metal bodies comprising a rotary

mold substantially closed at one end and open at the other end, means for supporting said mold for movement about an axis adjacent the closed end thereof, provisions adjacent the open end of the mold for moving the same about said axis, and charging means for said mold at said open end.

39. An apparatus for centrifugally casting hollow metal bodies comprising a rotary mold, means for supporting the same for movement between a substantially horizontal position and a position inclined to the horizontal, the said supporting means including mechanism for removably positioning the mold and adapted to permit rapid replacement of a poured mold by a mold to be poured, means for charging molten metal into the mold when the latter is in the inclined position, and provisions for moving the mold to the horizontal position while the metal is still in a fluid condition.

40. An apparatus for centrifugally casting hollow metal bodies comprising a rotary mold mounted for movement between a substantially horizontal position and a position inclined to the horizontal, means for rotating the mold including mechanism for permitting removal of the same for mold replacement, and means for charging molten metal into the mold when the latter is in the inclined position, and provisions for moving the mold to the horizontal position while the metal is in a fluid condition.

41. An apparatus for centrifugally casting hollow metal bodies comprising a rotary mold, means for supporting the same for movement about an axis adjacent one end thereof, the said supporting means including mechanism for removably positioning the mold and adapted to permit rapid replacement of a poured mold by a mold to be poured, and provisions for moving the mold about said axis.

42. An apparatus for centrifugally casting hollow metal bodies comprising a rotary mold, means for supporting the same for movement about an axis adjacent one end thereof, means for rotating the mold including mechanism for permitting removal of the mold for mold replacement, and provisions for moving the mold about the said axis.

43. An apparatus for centrifugally casting hollow metal bodies comprising a rotary mold, a supporting frame therefor, means for moving the supporting frame with the mold between inclined and horizontal positions, and a prime mover mounted upon the frame and having a driving connection with the mold.

44. An apparatus for centrifugally casting hollow metal bodies comprising a rotary mold, a supporting frame therefor, means for moving the supporting frame with the

5 mold between inclined and horizontal positions, and a prime mover axially aligned with the mold mounted on the frame and a detachable coupling means between the prime mover and the mold.

45. An apparatus for centrifugally casting hollow metal bodies comprising a rotary mold, a supporting frame therefor, mechanism for removably holding the mold on the frame and adapted to permit replacement of a poured mold by a mold to be poured, means for moving the supporting frame with the mold between inclined and horizontal positions, and a prime mover mounted upon the frame and having a driving connection with the mold.

46. An apparatus for centrifugally casting hollow metal bodies comprising a rotary mold substantially closed at one end, means for supporting the same including mechanism for removably holding the mold and adapted to permit replacement of a poured mold by a mold to be poured, and means for rotating the mold including a prime mover arranged co-axially with said mold and a detachable connection between the prime mover and the closed end of the mold.

47. An apparatus for centrifugally casting hollow metal bodies comprising a rotary mold, means for supporting the same including mechanism for removably holding the mold and adapted to permit replacement of a poured mold by a mold to be poured, and means for rotating the mold including an axially movable electric motor aligned with the axis of the mold and a separable coupling connecting the motor and the mold.

48. An apparatus for centrifugally casting hollow metal bodies comprising a rotary mold substantially closed at one end and having an opening at the other end, and means for charging the mold with molten metal through said opening, the said means including a pouring spout projecting into the mold through the lower portion only of said opening and arranged to permit the upper portion of the opening to remain unobstructed for the free egress of hot gases from the mold.

49. An apparatus for centrifugally casting hollow metal bodies comprising a rotary mold having an opening at one end thereof, and means for charging the mold with molten metal through said opening, the said means including a pouring spout substantially semicircular in cross section projecting into the mold opening at the lower half thereof and arranged to permit the upper half of the opening to remain unobstructed for the free egress of hot gases from the mold.

50. An apparatus for centrifugally casting hollow metal bodies comprising a rotary

65 mold having a bell-mouth end mounted for movement between a substantially horizontal position and a position inclined to the horizontal, means for charging molten metal into the end opposite the bell-mouth end and towards the bell-mouth end of the mold 70 when the mold is in the inclined position, and provisions for rapidly moving the mold to the horizontal position while the metal is still in a fluid condition, whereby an even distribution throughout the casting and including the bell end thereof is obtained.

51. In the art of centrifugally casting hollow metal bodies having bell ends, the method which consists in providing a rotary mold having a bell shaped structure at one 80 end and a pouring opening at the other end, in charging molten metal into the open end and toward the bell shaped end while the mold is rotating and in imparting a further movement to the mold other than a rotary movement to uniformly distribute the molten metal throughout the body of the mold.

52. In the art of centrifugally casting hollow metal bodies having bell ends, the 90 method which consists in providing an elongated rotary mold having a substantially closed bell shaped structure at one end and a pouring opening at the other end, in charging molten metal into the open end towards the well shaped end of the mold while the latter is rotating, and in imparting a tilting movement to the mold to uniformly distribute the molten metal throughout the body of the mold.

53. An apparatus for centrifugally casting molten metal bodies having bell ends, comprising a rotary mold having a bell shaped structure at one end and a pouring opening at the other end and means for uniformly distributing molten metal throughout the body of the mold comprising means for rotating the mold and means for imparting to the mold a movement supplemental to the rotating movement thereof.

54. An apparatus for centrifugally casting molten metal bodies having bell ends, comprising a rotary mold having a bell shaped structure at one end and a pouring opening at the other end and means for uniformly distributing molten metal throughout the body of the mold comprising means for rotating the mold and means for moving the mold from an inclined to a horizontal position while the metal is in a molten condition.

55. An apparatus for centrifugally casting hollow metal bodies comprising a rotary mold, means for supporting the same including mechanism for removably holding the mold and adapted to permit replacement of a poured mold by a mold to be poured, and means for rotating the mold including

an axially movable motor aligned with the axis of the mold and a flexible coupling connecting the motor and the mold.

56. An apparatus for centrifugally casting hollow metal bodies comprising a rotary mold, means for supporting the same including mechanism for removably holding the mold and adapted to permit replacement of a poured mold by a mold to be poured, and means for rotating the mold including a driving means arranged coaxially with said mold and a flexible detachable connection between the driving means and the mold.
57. In the art of centrifugally casting hollow metal bodies, the method which consists in charging a rotary mold with molten metal and in moving the rotary mold from a tilted to a substantially horizontal position while the metal is in a fluid condition.
58. In the art of centrifugally casting hollow metal bodies, the method which consists in rotating a charged mold about an axis and in moving the mold about a horizontal axis normal to the first mentioned axis while the metal is in a fluid condition.
59. In the art of centrifugally casting hollow metal bodies, the step in the method which consists in moving a rotary mold containing molten metal from a tilted to a substantially horizontal position while the metal is still in a fluid condition.
60. In the art of centrifugally casting hollow metal bodies, the method which consists in charging a rotary green sand mold having a membranous facing with molten metal and in moving the rotary mold from a tilted to a substantially horizontal position while the metal is in a fluid condition.
61. An apparatus for centrifugally casting hollow metal bodies comprising a rotary mold mounted for movement between a substantially horizontal position and a position inclined to the horizontal, and provisions for quickly moving the mold containing a

charge of molten metal from the inclined to the substantially horizontal position while the metal is still in a fluid condition.

62. An apparatus for centrifugally casting hollow metal bodies comprising a rotary mold, a supporting frame therefor, the said supporting frame being mounted for movement about an axis located adjacent an end of the mold so that the mold is arranged on one side of said axis, and a driving means for the mold mounted on the frame and arranged on the other side of said axis.

63. An apparatus for centrifugally casting hollow metal bodies comprising a rotary mold, a supporting frame therefor, the said supporting frame being mounted for movement about an axis located adjacent an end of the mold so that the mold is arranged on one side of said axis, and a prime mover for the mold mounted on the frame and arranged on the other side of said axis.

64. In the art of centrifugally casting hollow metal bodies, the method which consists in charging a mold with molten metal, in rotating the said mold and in manipulating the rotating mold while the metal is in a fluid condition to cause the bulk of the metal to flow towards one end of the mold and to then uniformly distribute itself throughout the body of the mold.

65. In the art of centrifugally casting hollow metal bodies, the method which consists in charging a mold with molten metal, in rotating the said mold and in imparting a further movement to the mold other than a rotary movement while the metal is in a fluid condition to cause the bulk of the metal to flow towards one end of the mold and to then uniformly distribute itself throughout the body of the mold.

Signed at New York city, in the county of New York and State of New York, this 21st day of Feb., A. D., 1923.

WILLIAM D. MOORE.